

## UNITED STATES PATENT OFFICE

FRITZ STÄBLEIN, OF ESSEN, GERMANY, ASSIGNOR TO FRIED. KRUPP AKTIENGESELLSCHAFT, OF ESSEN-ON-THE-RUHR, GERMANY

## IRON-NICKEL ALLOY

No Drawing. Application filed October 31, 1928, Serial No. 316,356, and in Germany December 24, 1927.

Nickel-iron alloys that contain about 50 to 85 per cent of nickel and more particularly those containing 78.5 per cent of nickel, possess a high initial permeability, that means

5 the proportion B:H of these alloys has a value, even with quite small field strengths, which is a multiple of the corresponding value of quite soft iron sorts. An undesired property of these alloys, however, consists 10 in the fact that in order to acquire their highest initial permeability they must be subjected to rather a complicated heat treatment. With the above-indicated nickel-iron alloy containing 78.5 per cent of nickel the heat 15 treatment required consists e. g. in heating the alloy to 900 degrees C. and cooling it first slowly to 600 degrees C. and then as quickly as possible to room temperature. With a nickel-iron alloy, however, that contains about 50 per cent of nickel, the best heat 20 treatment consists in glowing it a comparatively long time at about 1100 degrees C. and thereupon cooling it slowly.

A further unfavourable property of the indicated nickel-iron alloys is their small specific resistance which with the nickel-iron alloy containing 50 per cent of nickel amounts to about 0.47 Ohm. mm<sup>2</sup>/m and with that containing 78.5 per cent of nickel to 25 about 0.22 Ohm. mm<sup>2</sup>/m and results in high eddy-current losses and their consequences (differently great decrease of the apparent permeability with different alternating current frequencies, and distortions resulting 30 therefrom).

Now the subject-matter of the invention is an alloy which besides iron contains about 33 to 48 per cent of nickel and 0.3 to 3 per cent of silicon, the invention further consisting in 35 employing these alloys and alloys known per se which besides iron contain about 33 to 48 per cent of nickel and 0.3 to 5 per cent of silicon, to produce articles that must possess great initial permeability. Iron-nickel alloys of these compositions possess besides a 40 specific resistance of about 0.85 to 0.9 Ohm. mm<sup>2</sup>/m (that is four times that of the nickel-iron alloy containing 78.5 per cent of nickel), an initial permeability of the order 2000 to 45 3000, and a saturation intensity of about 50

11000 lines of force in each cm<sup>2</sup>, which is about equal to the saturation intensity of the nickel-iron alloy which contains 78.5 per cent of nickel.

The fact that the percentage of nickel is 55 considerably lower in the alloys indicated above than in the known nickel-iron alloys which possess high initial permeability affords the further advantage of the former being much cheaper than the latter, despite 60 their good electric and magnetic properties. Furthermore, the fact that the good electric and magnetic properties were obtained despite the low percentage of nickel proves that a deciding influence has to be attached to the 65 addition of silicon. Tests made with two iron-nickel alloys each containing 40 per cent of nickel but one of which contained 2 per cent of silicon while the other did not contain silicon, proved that the silicon-iron-nickel alloy 70 possesses an initial permeability of an average increase of 1000 units.

The impurities entering the alloys in the producing process are of no consequence in practice.

What I claim and desire to secure by Letters Patent, is:—

1. An iron-nickel alloy containing about 33 to 48 per cent of nickel, 0.3 to 3 per cent of silicon, and the remainder iron.
2. Articles of high initial permeability consisting of about 33 to 48 per cent of nickel, 0.3 to 5 per cent of silicon, and the remainder iron.
3. A magnetic material which comprises as 85 an essential component a composition containing 33 to 48% of nickel, 0.3 to 5% of silicon and the remainder iron, such composition having high initial permeability and high specific resistance.

The foregoing specification signed at Cologne, Germany, this 15th day of October, 1928.

FRITZ STÄBLEIN.